

M. ALISSOFF.

Copying Pad.

No. 231,517.

Patented Aug. 24, 1880.



Witnesses

C. J. Nottingham  
J. O. McCleary.

Michael Alisoff  
by his Attorneys  
Howson and Son

# UNITED STATES PATENT OFFICE.

MICHAEL ALISOFF, OF ST. PETERSBURG, RUSSIA, ASSIGNOR TO CHARLES GEORGE KLEBERG, OF LONDON.

## COPYING-PAD.

SPECIFICATION forming part of Letters Patent No. 281,517, dated August 24, 1880.

Application filed September 17, 1879. Patented in Belgium June 16, 1879, in Russia July 2, 1879, in France September 3, 1879, and in England February 25, 1880.

*To all whom it may concern:*

Be it known that I, MICHAEL ALISOFF, a subject of the Emperor of Russia, and a resident of St. Petersburg, Russia, have invented 5 an Improved Copying Pad or Matrix, for which I have obtained Belgian Letters Patent June 16, 1879, and of which the following is a specification, reference being had to the accompanying drawing.

10 My invention relates to the methods of obtaining a number of fac-simile copies of written or printed matter by writing or printing the original copy with aniline or specially-prepared inks, and then transferring the impression to a pad or matrix having a prepared surface, from which a number of impressions on ordinary paper may be obtained without inking the printing-surface thus prepared.

15 The object of my invention is to produce an improved transfer pad or matrix for this purpose; and this object I attain by preparing the surface to which the original writing or printing is to be transferred in the following manner:

20 I coat sized or unsized paper on one side with a composition consisting of animal glue, glycerine, and water in the following proportions: about eight pounds of animal glue and two pounds of glycerine and sufficient water—

25 say about twenty pounds—to give the composition the desired consistency. To this about two pounds of soap may be added, and also, if desired, two pounds of baryta or other white insoluble material, to give more consistency

30 and gloss to the composition. Whether either of these two last substances are used or not, a solution of tannin should be added to the mixture, in quantity—say about five pounds of tannin solution—sufficient to prevent the composition, when applied to the paper, from becoming sticky; or, if preferred, the paper which has been coated with a composition of the above ingredients without the tannin may be washed with a solution of tannin.

35 The paper to which the composition is to be applied may be of any suitable thickness, and if not transparent may be made so, if desired, by any of the ordinary and well-known means. To transfer to this surface the original matter

printed or written in prepared aniline ink, I 50 place a sheet, A, of the above prepared paper on a sheet, B, of damp flannel or cloth laid on a zinc plate or on oil-paper, C. The surface of the prepared paper, which I term "polygraphic" paper, is then sponged with clean 55 water, or in hot weather, with water containing a little alum, and the original written or printed sheet is then laid, face downward, on the polygraphic paper. Then another piece of damp flannel or cloth and a zinc plate or oil-paper are laid on the top, and the whole pile subjected to pressure in an ordinary copying-press or by other suitable means. When the pile is taken out of the press and the original detached from the polygraphic paper, it will 60 be found that the written or printed matter 65 has been transferred to the paper.

To obtain copies or impressions from the printing-surface thus formed, after removing the original, I place a sheet, D, of ordinary 70 paper, damp or dry, on the surface of the prepared sheet, in place of the detached original, and proceed in the same way as in transferring to the polygraphic or prepared sheet. In this manner I can obtain about forty copies by repeating the operation.

If copies or transfers are to be taken from two, four, six, or eight pages at once, I place a sheet of wet polygraphic paper on each page, with damp flannels and zinc plates between 75 the leaves of polygraphic paper, and proceed in the manner described above.

The inks with which the original is to be written or printed, and which I call "polygraphic" inks, are prepared as follows: To 80 make the writing-inks, I dissolve about one pound of aniline in about one and a quarter pound of alcohol, and when dissolved I add as much water to it as may be necessary to make it sufficiently fluid. The ink can then 85 be bottled for use.

To prepare polygraphic printing-ink, I take one pound of aniline and one pound of glycerine, and boil them until the aniline is dissolved and the composition has sufficient consistency 90 to be used as printer's ink.

The polygraphic printing-ink is more particularly useful for printing letter-heads, bill-

heads, circulars, &c., so that if polygraphic ink be used for both the printing and writing the copies or impressions taken will include both written and printed matter.

5 In using or preparing the polygraphic ink the hands are apt to become stained. These stains can be readily removed by a solution of tartaric acid in strong alcohol.

I do not desire to claim in this application 10 the method of obtaining copies by causing an absorbent gelatinous surface to take an impression from the original, and then pressing sheets of paper (damped or not) on this prepared surface; but

15 I claim as my invention—

The within-described composition for a matrix or pad for transfer-copying, consisting of animal glue, glycerine, water, and tannin solution, in about the following proportions: eight parts of animal glue, two parts of glycerine, five parts of tannin solution, and water sufficient to give the composition the desired consistency.

In testimony whereof I have signed my name to this specification in the presence of two sub- 20 scribing witnesses.

MICHAEL ALISSOFF.

Witnesses:

N. TSHERIALOFF,  
L. VOSS.